

Patented Jan. 21, 1947

2,414,620

# UNITED STATES PATENT OFFICE

2,414,620

## CATALYTIC DEHYDROISOMERIZATION OF FIVE MEMBERED ALICYCLIC RING HYDROCARBONS HAVING SIX OR MORE CARBON ATOMS PER MOLECULE TO AROMATIC HYDROCARBONS

Robert A. Trimble, El Cerrito, Calif., assignor to  
Shell Development Company, San Francisco,  
Calif., a corporation of Delaware

No Drawing. Application August 22, 1944,  
Serial No. 550,674

12 Claims. (Cl. 260—668)

1

This invention relates to the production of aromatic hydrocarbons and relates more particularly to the direct dehydroisomerization of five membered alicyclic ring compounds having at least six carbon atoms to the molecule to aromatic hydrocarbons. A particular aspect of the invention relates to the dehydroaromatization of methylcyclopentane to benzene.

Petroleum is becoming of increasing importance as a source of highly desirable aromatic hydrocarbons. Processes proposed heretofore for the production of aromatic hydrocarbons from petroleum include many directed to the separation of aromatic hydrocarbons originally present therein by such procedures as fractional distillation, solvent extraction, extractive distillation, etc. Other methods involve the step of thermally treating suitable hydrocarbons under drastic temperature conditions and subsequent separation of aromatic hydrocarbons from the pyrolysis product. Still other methods involve such steps as the catalytic cyclization of paraffinic hydrocarbons, for example, the catalytic cyclization of normal hexane to benzene, and the dehydrogenation of cycloparaffins of hydroaromatic structure such as, for example, the dehydrogenation of cyclohexane to benzene.

Many of these processes, although yielding substantial amounts of desirable aromatic hydrocarbons, often involve operations, the complexity and cost of which often render the process economically unfeasible. Others are rendered unattractive by relatively low yields. These processes are furthermore seriously handicapped by the fact that the particular hydrocarbons capable of conversion thereby in a single step operation to desired aromatic hydrocarbons are often more valuable as raw material for other processes. New methods enabling the conversion to aromatic hydrocarbons in a single step operation of individual hydrocarbons not efficiently converted heretofore in single step operations were therefore sought after. Such a process would enable not only the more efficient production of aromatic hydrocarbons but would render economically more attractive, and provide greater flexibility in the execution of, many other refinery operations influenced by, and often even dependent upon, the type of aromatic hydrocarbon production step employed.

It is an object of the present invention to provide an improved process for the more efficient production of aromatic hydrocarbons in a single step operation from readily available hydrocarbon materials. It is a further object of the inven-

2

tion to provide an improved process for the more efficient conversion of five membered alicyclic ring compounds having at least six carbon atoms to the molecule to aromatic hydrocarbons. A more specific object of the invention is the provision of an improved process for the direct dehydroaromatization of methylcyclopentane to benzene. Other objects and advantages of the invention will become apparent from the following detailed description thereof.

The five membered alicyclic ring compounds having at least six carbon atoms to the molecule contained in readily available hydrocarbon mixtures are a particularly suitable source material for the production of aromatic hydrocarbons. As shown above, certain cycloparaffins have heretofore been dehydrogenated to aromatic hydrocarbons. Cyclohexane, for example, has been catalytically dehydrogenated to benzene. Such processes, however, do not enable the utilization of five membered alicyclic ring compounds present in the charge and furthermore often involve the destruction of these materials to less desirable hydrocarbons. Other processes available heretofore, though enabling the conversion of certain of the five membered alicyclic ring compounds to aromatic hydrocarbons, generally involve a plurality of separate reactions. Methylcyclopentane is converted to benzene by successive steps involving, first, the isomerization of the methylcyclopentane to cyclohexane and thereafter, the separate dehydrogenation of the cyclohexane formed to benzene. Such a plurality of steps is often sufficiently costly and complex to render their practical application, as well as the execution of other processes carried out in conjunction therewith, highly impractical.

In accordance with the present invention the five membered alicyclic ring compounds having at least six carbon atoms to the molecule are converted to aromatic hydrocarbons in a single step operation. Methylcyclopentane is converted directly to benzene. The reaction mechanism involved, resulting in the direct, single step conversion of a cyclic hydrocarbon containing a five-membered alicyclic ring to a hydrocarbon containing a six-membered ring of aromatic character, is termed throughout the specification and appended claims "dehydroisomerization."

It has been found recently that the dehydroisomerization reaction is promoted by certain highly specific catalysts. Of the many dehydrogenation catalysts such as chromium oxide, tungsten oxide, vanadium oxide, titanium oxide, iron oxide, platinum, nickel, etc., the only catalyst so

far found enabling the execution of the reaction with relatively favorable yields is molybdenum oxide. Tungsten sulfide and molybdenum sulfide are found to exert to some degree a favorable effect upon the dehydroisomerization reaction. These sulfide catalysts have the highly advantageous attribute of being immune to poisoning by sulfur and the sulfur-containing materials often present as impurities in the hydrocarbon charge. The catalytic effect of the tungsten sulfide or molybdenum sulfide upon the dehydroisomerization reaction is, however, so slight as to render the production of aromatic hydrocarbons from cyclic hydrocarbons containing a five membered alicyclic ring with the aid of these catalysts 15 highly impractical.

It has now been found that the catalytic effect of tungsten sulfide and molybdenum sulfide upon the dehydroisomerization reaction is markedly influenced by the presence of nickel. It has furthermore been found that the presence of nickel in the tungsten or molybdenum sulfide within well defined concentrations enables the efficient direct dehydroisomerization of five membered alicyclic ring compounds having at least six carbon atoms to the molecule to aromatic hydrocarbons with high yields.

The catalysts comprising tungsten sulfide, or molybdenum sulfide, and a promotional amount of nickel are prepared in any of many suitable ways. Preferred promoted catalysts of the invention contain the nickel in the freshly prepared catalyst in the sulfided state. Particularly preferred catalysts comprise those prepared under conditions involving the precipitation of nickel in the sulfide form in the presence of sulfur compounds of tungsten or molybdenum. A preferred method of preparing the promoted catalysts of the invention is as follows:

To an ammonium thiotungstate solution, prepared from an ammoniacal aqueous tungstic acid solution with hydrogen sulfide, there is added an aqueous solution of nickel nitrate. A precipitate consisting largely of nickel sulfide forms. Dilute sulfuric acid is added until the hydrogen ion concentration of the resulting mixture, in terms of the pH values, is in the range of from about 1 to about 2. Tungsten is thereby precipitated as tungsten trisulfide. The precipitate is separated from the liquor by filtration and/or centrifuging. The resulting tungsten-nickel sulfides are dried and calcined at a temperature of from about 400 to about 425° C. in a hydrogen atmosphere, thereby effecting the conversion of tungsten trisulfide to tungsten disulfide.

The catalyst is employed as such in the form of lumps, pills, extrudates, or in any other suitable shape or form assuring efficient contact between catalyst and reactants during use. The catalyst may furthermore be deposited upon, or diluted with, suitable solid support material comprising, for example, porous adsorptive materials such as carbon, Activated Alumina, bauxite, adsorptive clays, magnesia, etc.

As stated above, the degree of catalytic effect upon the dehydroisomerization reaction is dependent upon the concentration of nickel in the catalyst. It has been found that superior catalysts resulting in the attainment of more efficient operation with high yields of the desired aromatic hydrocarbon comprise those having a nickel content in the range of from about 2% to about 15% and preferably from about 4% to about 11% by weight of the total metal content of the catalyst. Though the utilization of catalysts containing

somewhat greater or lesser amounts of nickel is contemplated within the scope of the invention such catalysts are, however, not generally preferred because their lesser catalytic effect upon the dehydroisomerization reaction generally renders impractical their utilization in large scale operation. Catalysts of unusual activity with respect to the dehydroisomerization reaction are those having a nickel content of about 7%. By the term "total metal content" of the catalyst as used throughout the specification and claims is meant the summation of the total ultimate content of tungsten and/or molybdenum and nickel in the catalyst regardless of the manner or proportion in which any or all of these metals are combined with other chemical elements such as, for example, sulfur, in the catalyst. Determination of the nickel concentration within the prescribed range necessary to attain a catalyst of desired dehydroisomerization activity is therefore not only independent of the elements chemically combined with the metal content of the catalyst but is also independent of the composition or amount of solid support or diluent material added to the catalyst either during or after its manufacture.

In accordance with the process of the invention the five membered alicyclic compounds having at least six carbon atoms to the molecule are contacted in the vapor phase with the catalyst in any suitable type of reactor enabling efficient contact of the catalyst with the hydrocarbon charge. Such reactors may utilize the catalyst in the form of stationary or moving beds or even in a suspended or fluidized state. Five membered alicyclic ring compounds having at least six carbon atoms to the molecule which are capable of undergoing conversion to aromatic hydrocarbons in accordance with the invention include the hydrocarbons containing a pentacarbocyclic ring of saturated or unsaturated character in which at least one of the hydrogen atoms attached to a carbon atom in the ring is replaced by an alkyl or alkenyl group. Such five membered alicyclic ring compounds comprise cyclopentane and cyclopentene in which at least one of the hydrogen atoms is replaced by an alkyl or alkenyl group, for example, methylcyclopentane, ethylcyclopentane, propylcyclopentane, isopropylcyclopentane, dimethylcyclopentane, trimethylcyclopentane, tetramethylcyclopentane, 1-methyl-2-ethylcyclopentane, diethylcyclopentane, methylene-cyclopentane, cyclopentylacetylene, 1-methyl-2-isopropenyl cyclopentane, 1-methyl-2-isopropylidene-cyclopentane, 3-methyl-1-methylene-cyclopentane, ethylidene-cyclopentane, 1-methyl-2-ethylidene cyclopentane, 1,1,2-trimethyl-3-methylene cyclopentane, 1-methyl-1-cyclopentene, 3-methyl-1-cyclopentene, 1,2-dimethyl-1-cyclopentene, 3,3 - dimethyl-1-cyclopentene, 1-ethyl-1-cyclopentene, 1-isopropyl - 1 - cyclopentene, 1,2,3-trimethyl-1-cyclopentene, 1,3 - dimethyl-2-ethyl-1-cyclopentene, 1-vinyl-1-cyclopentene, 1-propenyl-1-cyclopentene, 1-methyl-2-isopropenyl-1-cyclopentene, etc. The hydrocarbon charge to the reaction zone may consist of essentially only one five membered alicyclic ring compound having at least six carbon atoms to the molecule or may comprise more than one such cyclic hydrocarbon capable of direct dehydroisomerization to aromatic hydrocarbons. The hydrocarbon charge may furthermore contain other hydrocarbons capable or not of undergoing conversion under conditions of execution of the dehydroisomerization reaction. Suitable hydro-

carbon charge material comprises hydrocarbon mixtures of relatively narrow boiling range containing at least one five membered alicyclic compound having at least six carbon atoms to the molecule, such as are obtained by fractionation, solvent extraction, extractive distillation, etc., of readily available hydrocarbon mixtures containing the cyclic hydrocarbons. A particularly desirable charge comprises a concentrate of the five membered alicyclic compound having at least six carbon atoms to the molecule such as, for example, a methylcyclopentane concentrate, obtained by fractionation of hydrocarbon mixtures such as naphthenic straight run gasolines or other suitable methylcyclopentane-containing hydrocarbon mixtures.

The hydrocarbon charge is contacted with the catalyst under dehydroisomerizing conditions. Suitable dehydroisomerizing conditions include, for example, a temperature in the range of from about 400 to about 600° C. and preferably in the range of from about 475 to about 525° C. The reaction is executed under superatmospheric pressure, for example, in the range of from about 5 to about 100 atmospheres. Higher pressures may be resorted to. Hydrogen is introduced into the reaction zone in amounts sufficient to maintain a partial pressure of hydrogen in the reaction zone of from about 1 atmosphere to about 100 atmospheres and preferably from about 5 to about 45. Hydrogen is introduced into the reaction zone in admixture with the hydrocarbon charge or may be separately introduced in part, or in its entirety, at one or several points along the length of the reaction zone. Sulfur, or sulfur-containing compounds, present in the reactants exert a favorable influence upon the catalyst life. Small amounts of sulfur, for example, in the form of hydrogen sulfide, are therefore preferably added to the hydrocarbon charge or to the hydrogen passed to the reaction zone. In a preferred method of carrying out the process, sulfur present in the reaction products, for example, in the form of hydrogen sulfide, is recycled, at least in part, together with the hydrogen to the reaction zone. The contact time is maintained within a range of, for example, from about 4 seconds to about 500 seconds.

Under the above-defined conditions five membered alicyclic ring compounds having at least six carbon atoms to the molecule are converted efficiently in a single step operation to aromatic hydrocarbons. Thus, methylcyclopentane is converted to benzene with high yields and in the absence of any substantial amount of undesirable side reactions. Regeneration of the catalyst is effected by burning off deposited carbonaceous material with the aid of oxygen or oxygen containing gases in the usual manner. Excessive amounts of sulfur removed in this operation are replaced by treatment of the catalyst in situ with hydrogen sulfide.

The following examples are illustrative of the efficiency with which five membered alicyclic ring compounds having at least six carbon atoms to the molecule are dehydroisomerized to aromatic hydrocarbons in a single step operation in accordance with the invention.

#### EXAMPLE I

Methylcyclopentane was contacted under dehydroisomerizing conditions with a catalyst consisting of unpromoted tungsten sulfide. In three further separate operations methylcyclopentane was contacted under the same dehydroisomeriz-

ing conditions with catalysts consisting of precipitated mixtures of tungsten sulfide and nickel sulfide prepared as above. The nickel content of each of the catalysts in percent by weight, and the benzene content in percent by volume in the reaction product of each operation, are given in Table A. The dehydroisomerizing conditions used in each of the runs were as follows:

10 Temperature 490° C.  
Pressure 20 atm.  
Contact time 100 secs.  
Mol ratio of added hydrogen to feed 3.0

15

Table A

| Run | Catalyst                                                    | Nickel content in per cent by weight of total metal content of catalyst | Benzene in product per cent by volume |
|-----|-------------------------------------------------------------|-------------------------------------------------------------------------|---------------------------------------|
| 20  | 1. Tungsten sulfide.<br>2. Tungsten sulfide-nickel sulfide. | 0<br>5.05                                                               | 9<br>45                               |
| 25  | 3. do.<br>4. do.                                            | 7.05<br>13.75                                                           | 81<br>19                              |

#### EXAMPLE II

Methylcyclopentane was contacted under the dehydroisomerizing conditions of Example I with a catalyst consisting of unpromoted molybdenum sulfide. In a separate operation under identical dehydroisomerizing conditions methylcyclopentane was contacted with a catalyst consisting of molybdenum sulfide and nickel sulfide having a nickel content of 8.5% by weight based on the total metal content of the catalyst. The benzene content of the product obtained with the unpromoted molybdenum sulfide catalyst was only 8 percent by volume whereas the benzene content of the product obtained with the molybdenum sulfide-nickel sulfide catalyst amounted to 34 percent by volume.

I claim as my invention:

1. A process for the direct conversion of methylcyclopentane to benzene which comprises contacting methylcyclopentane under dehydroisomerizing conditions with a catalyst comprising a member of the group consisting of tungsten sulfide and molybdenum sulfide containing about 7 per cent by weight of nickel based on the total metal content of said catalyst, said nickel being in the sulfided state.

2. A process for the direct conversion of methylcyclopentane to benzene which comprises contacting methylcyclopentane under dehydroisomerizing conditions with a catalyst comprising a member of the group consisting of tungsten sulfide and molybdenum sulfide containing a promoting amount of nickel in the range of from about 4 to about 11 per cent by weight of the total metal content of the promoted catalyst, said nickel being in the sulfided state.

3. A process for the production of benzene from a mixture of hydrocarbons containing methylcyclopentane which comprises contacting said hydrocarbon mixture under dehydroisomerizing conditions with a catalyst comprising a member of the group consisting of tungsten sulfide and molybdenum sulfide containing a promoting amount of nickel in the range of from about 2 to about 15 percent by weight of the total metal content of the promoted catalyst, said nickel being in the sulfided state, thereby effecting the dehydroisomerization of methylcyclopentane to benzene.

4. A process for the direct conversion of methylcyclopentane to benzene which comprises contacting methylcyclopentane under dehydroisomerizing conditions with a catalyst consisting essentially of tungsten sulfide containing about 7 per cent by weight of nickel based upon the total metal content of said catalyst, said nickel being in the sulfided state.

5. A process for the production of benzene from a mixture of hydrocarbons containing methylcyclopentane which comprises contacting said hydrocarbon mixture under dehydroisomerizing conditions with a catalyst consisting essentially of tungsten sulfide containing a promoting amount of nickel in the range of from about 2 to about 15 percent by weight of the total metal content of the promoted catalyst, said nickel being in the sulfided state, thereby effecting the direct conversion of methylcyclopentane to benzene.

6. A process for the production of benzene from a mixture of hydrocarbons containing methylcyclopentane which comprises contacting said hydrocarbon mixture under dehydroisomerizing conditions with a catalyst consisting essentially of molybdenum sulfide containing a promoting amount of nickel in the range of from about 2 to about 15 percent by weight of the total metal content of the promoted catalyst, said nickel being in the sulfided state, thereby effecting the direct conversion of methylcyclopentane to benzene.

7. A process for the direct conversion of cycloparaffins of non-hydroaromatic structure having at least six carbon atoms in the molecule and containing five carbon atoms in the ring to aromatic hydrocarbons which comprises contacting said cycloparaffins of nonhydroaromatic structure under dehydroisomerizing conditions with a catalyst comprising a member of the group consisting of tungsten sulfide and molybdenum sulfide containing about 7 per cent by weight of nickel based on the total metal content of said catalyst, said nickel being in the sulfided state, thereby effecting the direct conversion of cycloparaffins of nonhydroaromatic structure to aromatic hydrocarbons.

8. A process for the direct conversion of five membered alicyclic ring compounds having at least six carbon atoms to the molecule to aromatic hydrocarbons which comprises contacting said five membered alicyclic ring compounds under dehydroisomerizing conditions with a catalyst comprising a member of the group consisting of tungsten sulfide and molybdenum sulfide containing a promoting amount of nickel in the range of from about 4 to about 11 per cent by weight of the total metal content of the promoted catalyst, said nickel being in the sulfided

state, thereby effecting the direct conversion of said five membered alicyclic ring compounds to aromatic hydrocarbons.

9. A process for the production of aromatic hydrocarbons from a hydrocarbon mixture containing five membered alicyclic ring compounds having at least six carbon atoms to the molecule which comprises contacting said hydrocarbon mixture under dehydroisomerizing conditions with a catalyst comprising a member of the group consisting of tungsten sulfide and molybdenum sulfide containing a promoting amount of nickel in the range of from about 2 to about 15 percent by weight of the total metal content of the promoted catalyst, said nickel being in the sulfided state, thereby effecting the direct conversion of said five membered alicyclic ring compounds to aromatic hydrocarbons.

10. A process for the direct conversion of cycloparaffins of nonhydroaromatic structure having at least six carbon atoms in the molecule and containing five carbon atoms in the ring to aromatic hydrocarbons which comprises contacting said cycloparaffins of nonhydroaromatic structure under dehydroisomerizing conditions with a catalyst consisting essentially of tungsten sulfide containing a promoting amount of nickel in the range of from about 4 to about 11 per cent by weight of the total metal content of the promoted catalyst, said nickel being in the sulfided state.

11. A process for the production of aromatic hydrocarbons from a hydrocarbon mixture containing five membered alicyclic ring compounds having at least six carbon atoms to the molecule which comprises contacting said hydrocarbon mixture under dehydroisomerizing conditions with a catalyst consisting essentially of tungsten sulfide containing a promoting amount of nickel in the range of from about 2 to about 15 percent by weight of the total metal content of the promoted catalyst, said nickel being in the sulfided state, thereby effecting the dehydroisomerization of said five membered alicyclic ring compounds to aromatic hydrocarbons.

12. A process for the production of aromatic hydrocarbons from a mixture of hydrocarbons containing five membered alicyclic ring compounds having at least six carbon atoms to the molecule which comprises contacting said hydrocarbon mixture under dehydroisomerizing conditions with a catalyst consisting essentially of molybdenum sulfide containing a promoting amount of nickel in the range of from about 2 to about 15 percent by weight of the total metal content of the promoted catalyst, said nickel being in the sulfided state, thereby effecting the dehydroisomerization of said five membered alicyclic ring compounds to aromatic hydrocarbons.

ROBERT A. TRIMBLE.